

No. 861,650.

PATENTED JULY 30, 1907.

W. E. HASSAM.

ARTIFICIAL STRUCTURE AND PROCESS OF MAKING THE SAME.

APPLICATION FILED NOV. 30, 1906.

*Fig. 1*



*Fig. 2*



Witnesses:

C. H. Hassan  
E. M. Allen.

For Inventor:  
Walter E. Hassan  
by attorneys  
Lindquist & Lindquist

# UNITED STATES PATENT OFFICE.

WALTER E. HASSAM, OF WORCESTER, MASSACHUSETTS, ASSIGNOR TO HASSAM PAVING COMPANY, OF WORCESTER, MASSACHUSETTS, A CORPORATION OF MASSACHUSETTS.

## ARTIFICIAL STRUCTURE AND PROCESS OF MAKING THE SAME.

No. 861,650.

Specification of Letters Patent.

Patented July 30, 1907.

Application filed November 30, 1906. Serial No. 345,729.

*To all whom it may concern:*

Be it known that I, WALTER E. HASSAM, a citizen of the United States, residing at Worcester, in the county of Worcester and State of Massachusetts, have invented 5 a new and useful Artificial Structure and Process of Making the Same, of which the following is a specification.

My invention relates to an artificial structure capable of use for foundations, walls, abutments, columns, 10 floors, etc., but especially adapted for pavements for roads, sidewalks, and the like.

In a prior patent granted to me on the first day of May 1906, No. 819,652 I have described a structure in which, broken stone, gravel, or the like has been 15 placed on the bottom of an excavation and rolled to compact the same, and the broken stone or gravel has been treated with a grouting or the like, subsequent to its rolling, and a suitable wearing surface has been placed thereon.

20 The principal object of this invention is to provide for improving the surface layer, and the improved surface layer can be used either with those constructions and methods which involve the use of previously coated stone, or with that which is carried out with 25 uncoated stone afterwards grouted.

Reference is to be had to the accompanying drawings, in which

Figure 1 is a sectional view of a portion of an excavation with uncoated stone placed therein, ready to be 30 compressed, and Fig. 2 is a similar view of the structure as completed constituting a pavement.

In carrying out the invention, the bottom of the excavation is preferably rolled, and then a layer of broken stone or gravel *a* is placed therein and rolled 35 hard. For example, it may be eight inches deep when originally placed in position, and rolled or compressed until it is six inches deep.

In the preferred embodiment of the invention, the stone is placed in position in an uncoated state and 40 rolled hard or compressed and thereafter grouted with a more or less thin cement grouting *b* to fill all the voids among the stone. The invention also may be carried out in connection with the method which consists in coating the stones before they are placed in the excava-

tion and rolled. In either event, a layer of grouting 45 *c* is placed on the layer of stones. If previously coated stones are used, this surfacing layer *c* has to be applied as a separate step of the process, but if uncoated stones are employed, the grouting is poured down upon them, not only until it fills the voids, but until the layer *c* is 50 produced, so that this is a continuation of the grouting *b* and homogeneous therewith.

In order to produce a suitable surface on top of the pavement or other structure which is being made, uncoated fine or pea stones are rolled into the layer *c* before 55 the cement has a chance to set or harden. The top layer *c* however, may be formed of a mixture of sand, cement, and fine pea stones preferably in substantially equal proportions, and a suitable amount of water and applied to the top of the layer of hard rolled 60 stones.

While I have illustrated and described a preferred embodiment of my invention, I am aware that modifications may be made therein without departing from the spirit of the invention as expressed in the claims. 65

Having thus described my invention, what I claim is:

1. An artificial structure comprising a foundation layer of hard rolled stone having grouting filling the voids therein and a surface layer comprising a continuation of 70 said grouting containing fine stones compressed into its surface.

2. A road or pavement consisting of a bottom layer of hard rolled uncoated stone, a grouting of cement placed upon said stone and filling all the voids therein, and a 75 top layer of smaller uncoated stones compressed into the surface of said grouting before it sets.

3. A road or pavement consisting of a bottom layer of stone, a grouting placed upon said stone and filling all the voids therein, and a top layer of smaller uncoated stone 80 compressed into the surface of said grouting before it sets.

4. The method of making a pavement which consists in rolling uncoated stone, placing a thin grouting thereupon, allowing the grouting to run down and fill the voids in the 85 layer of stones, and compressing fine uncoated stones into said grouting before it sets.

In testimony whereof I have hereunto set my hand, in the presence of two subscribing witnesses.

WALTER E. HASSAM.

Witnesses:

LOUIS W. SOUTHGATE.  
MARY E. REGAN.